

[54] PROCESS AND APPARATUS FOR  
CONTINUOUSLY PRODUCING SLUB YARN

[75] Inventors: **Kiyoshi Adachi**, Nagoya; **Iwao Miyashita**, Kasugai; **Kiyoto Haba**, Nagoya; **Kunio Shibata**, Nagoya; **Eizi Takahashi**, Toyoake, all of Japan

[73] Assignee: **Mitsubishi Rayon Co., Ltd.**, Japan

[22] Filed: Jan. 30, 1974

[21] Appl. No.: 437,796

[52] U.S. Cl. .... 57/34 B; 28/1.4; 28/72.12; 57/140 BY; 57/140 J; 57/157 F

[51] Int. Cl. .... D02G 1/16; D02G 3/04; D02G 3/34; D02G 3/40

[58] Field of Search ..... 57/34 B, 157 F, 140 J, 57/140 BY, 153, 164; 28/1.4, 72.12

## [56] References Cited

## UNITED STATES PATENTS

|           |        |                     |          |
|-----------|--------|---------------------|----------|
| 3,116,589 | 1/1964 | Edwards et al. .... | 57/157 F |
| 3,122,816 | 3/1964 | Rhoden.....         | 28/72.12 |

|           |         |                     |          |
|-----------|---------|---------------------|----------|
| 3,433,007 | 3/1969  | Myers .....         | 57/140 J |
| 3,474,613 | 10/1969 | Joarder et al. .... | 57/34 B  |

Primary Examiner—John Petrakes  
Attorney, Agent, or Firm—Armstrong, Nikaido & Wegner

[57]

## ABSTRACT

A slub yarn having a hand spun silk yarn-like appearance and feel to the hand is continuously produced from a multifilament yarn by feeding the multifilament yarn into a reduced pressure region formed in a hollow column at a predetermined feed rate while vigorously sucking air from the atmosphere through the region, agitating the multifilament yarn by the sucked air current to convert portions of the yarn into slubs consisting of portions of the yarn and/or the individual filaments entangled, intertwined, looped, bent and/or folded by action of the sucked air vortex or turbulent current, and delivering the resultant slub yarn from the reduced pressure region at a delivery rate lower than the feed rate.

32 Claims, 11 Drawing Figures



Fig. 1



Fig. 2



Fig. 3



Fig. 4



Fig. 5



Fig. 6



Fig. 7





**PROCESS AND APPARATUS FOR CONTINUOUSLY PRODUCING SLUB YARN**

The present invention relates to a process and apparatus for producing a multifilament fancy yarn, more particularly, it relates to a process and apparatus for continuously producing a multifilament slub yarn suitable for forming a silk shun tung-like fabric.

The term "silk shun tung" used here refers to a hand-made fabric of a hand spun silk yarn which is uneven in thickness. This hand spun silk yarn has slubs and knots formed thereon.

According to the general accepted idea, the principal purpose of weaving and knitting is to provide a fabric having a desired appearance and feel to the hand. In this regard, the silk fabric called shun tung received universal commendation when it appeared because of its grain, elegant and naive appearance and feel to the hand.

There have been attempts to produce an artificial filament fancy yarn having a hand spun silk yarn-like appearance and feel. In the most conventionally used of these attempts the yarn is produced, using a fancy twister, by intermittently twining a multifilament yarn about a multifilament core yarn to form slubs and then, bonding the slub-forming yarn and the core yarn with a multifilament bonding yarn. In the conventional method stated above, the resultant fancy yarn feels hard to the hand because the component yarns are firmly twisted. Accordingly, the fabric made of the conventional fancy yarn feels too hard even though the fabric has the shun tung-like appearance.

It is known from other attempts that the hand spun silk yarn-like fancy yarn is produced by feeding at least one multifilament yarn intermittently and at least one multifilament yarn continuously into a zone blown by a fluid jet. By the action of the fluid jet, the individual filaments in the yarns are entangled and, intertwined with each other. That is, the continuously fed yarn is converted to slubs formed on the intermittently fed yarn.

However, the known process stated above has the following disadvantages.

1. High cost in production, because two or more component multifilaments are necessary for producing only one fancy yarn.

2. Very complicated production apparatus, because one or more component yarns must be intermittently fed to the twister.

3. Undesirable formation of a wood grain-like pattern or tortoise shell pattern on the fabric, because the slubs are formed on the yarn at fixed intervals.

4. Low efficiency in energy utilization of the fluid jet.

5. Low production velocity.

An object of the present invention is to provide a process and apparatus for continuously producing slub yarns having a hand spun silk yarn-like appearance, a soft feel to the hand and high processability, with high efficiency and at a high production velocity.

The other object of the present invention is to provide a process and apparatus for continuously producing slub yarns having slubs firmly bundled on the yarn, using a simple slub-forming means.

The above-stated objects can be accomplished by the process and apparatus of the present invention. According to the process of the present invention, a slub yarn is continuously produced by the steps of providing a reduced pressure region by sucking air from the at-

mosphere through the region, feeding a multifilament yarn into the reduced pressure region at a predetermined feed rate while continuing to suck the air through the reduced pressure region, agitating the fed

5 yarn within the reduced pressure region by the action of the sucked air current to convert portions of the fed yarn into slubs consisting of entangled, intertwined and/or folded portions of said yarn and/or individual filaments in said yarn, and delivering the resultant slub

10 yarn from the reduced pressure region at a delivery rate lower than the feed rate.

The apparatus of the present invention comprises a slub-forming device comprising a hollow column having a yarn supply end plate with a yarn supply hole

15 formed thereon and a yarn delivery end plate with a yarn supply hole formed thereon, means for feeding a multifilament yarn into said slub-forming device at a predetermined feed rate, and means for delivering the slub yarn from said slub-forming device at a delivery

20 rate lower than the feed rate, the slub-forming device being connected at its periphery to a vacuum device through an air suction pipe.

When the multifilament yarn is fed into the reduced pressure region formed in the slub-forming device at a

25 feed rate higher than the delivery rate, the multifilament yarn is agitated by the action of air stream vigorously sucked from the atmosphere through the yarn supply and delivery holes into the reduced pressure region. As a result of the agitation, portions of the multi-

30 filament yarn and/or portions of individual filaments in the yarn are entangled, intertwined, folded and/or bent to form the slubs on the yarn. The portions of the yarn are converted into the slubs in response to the difference between the feed rate and the delivery rate. That

35 is, not all of the multifilament yarn is converted into slubs. While the multifilament yarn fed into the reduced pressure region is agitated by the action of the sucked air stream and vigorously moves throughout the region, some portions of the yarn or the individual filaments are rubbed with other portions of the yarn, other

40 filaments or the inside wall surface of the slub-forming device so as to produce static electricity thereon. This static electricity generated on some portions of the yarn or individual filaments can promote the entangle-

45 ment, intertwining bending and/or folding of the yarns and/or the individual filaments. The generation of the static electricity is effected irregular and at unfixed intervals of time on portions of the yarn or the individual filaments. This causes irregular distribution and un-

50 fixed lengths and thicknesses of the slubs.

The reduced pressure region is formed in a slub-forming device by vigorously sucking air with a vacuum device from the atmosphere through the yarn supply hole, yarn delivery hole and the slub-forming device.

55 The sucked air generates vigorous vortexes or turbulent currents in the slub-forming device. The vigorous air vortexes or turbulent currents can agitate the multifilament yarn to open it into separate individual filaments and entangle, intertwine, bend and/or fold the

60 individual filaments. The type and amount of the air vortexes or turbulent currents are in response to the type of slub-forming device and capacity of the vacuum device. The vacuum device usable for the apparatus of the present invention may be a vacuum pump, suction

65 fan or ejector.

In the process of the present invention, the multifilament yarn is preferably fed upward into the reduced pressure region and travels upward through the region

and then, the slub yarn is delivered upward from the region. However, the yarn may travel downward or laterally.

The features and advantages of the present invention will be apparent to persons acquainted with this type of fancy yarn upon reading the following descriptions and referring to the accompanying drawings, in which:

FIG. 1 shows an explanatory view of an embodiment of the apparatus of the present invention;

FIG. 2 shows an explanatory cross-sectional view of an embodiment of a slub-forming device with an air suction pipe, usable for the apparatus of the present invention;

FIG. 3 is an explanatory cross-sectional view of an embodiment of a slub-forming device with an air suction pipe and an air permeable partition disposed in the slub-forming device, usable for the apparatus of the present invention;

FIG. 4 is an explanatory cross-sectional view of an embodiment of a slub-forming device with an air suction pipe and an air permeable partition located in the air suction pipe, usable for the apparatus of the present invention;

FIG. 5 is an explanatory cross-sectional view of an embodiment of a slub-forming device with an air suction pipe, a yarn storage inner tube disposed in a yarn supply end portion of the slub-forming device and an air suction member located in a yarn delivery end portion of the slub-forming device, usable for the apparatus of the present invention;

FIG. 6 shows a cross-section of the air suction member shown in FIG. 5, along line VI—VI in FIG. 5;

FIG. 7 shows a cross-section of the slub-forming device shown in FIG. 5, along line VII—VII in FIG. 5;

FIG. 8 is an explanatory cross-sectional view of an embodiment of a slub-forming device with an air suction pipe, an air suction member, a yarn storage inner hollow column and an air vortex inner hollow column disposed between the air suction member and the yarn storage inner hollow column, usable for the apparatus of the present invention;

FIG. 9 shows a cross-section of the slub-forming device shown in FIG. 8, along line IX—IX in FIG. 8, and;

FIGS. 10 and 11 respectively show an explanatory view of an embodiment of the slub yarn produced in accordance with the present invention.

The process of the present invention may be carried out by the apparatus as shown in FIG. 1. In the drawing, a multifilament yarn 1 is taken from a yarn supply package 2 by means of a pair of feed rollers 3a and 3b and fed into a slub-forming device 4 at a predetermined feed rate. The slub-forming device 4 is connected to a vacuum device 5 through an air suction pipe 6 to define therein a reduced pressure region. When the vacuum device 5 is actuated, the reduced pressure region is formed in the slub-forming device 4, and air is vigorously sucked from the atmosphere into the slub-forming device 4. The sucked air produces a vigorous vortex or turbulent current in the slub-forming device. By the action of the sucked air current, the multifilament yarn is converted into a slub yarn 7 having slubs 7a while the multifilament yarn is in the slub-forming device 4. The slub yarn 7 is removed from the slub-forming device 4 by means of a delivery roller 8 at a delivery rate lower than the feed rate, and wound up into a yarn take up package 9.

As stated above, while the multifilament yarn 1 is in the slub-forming device 4, the yarn 1 is vigorously agi-

tated by the action of the air vortex or turbulent current. This agitation results in looping, bending, folding and opening of the multifilament yarn and entanglement, intertwining, looping, bending and folding of the separated individual filaments. These movements of the yarn and individual filaments cause the irregular formation of slubs on the yarn. That is, some portions of the multifilament yarn are converted to slubs having irregular length and thickness and such slubs are distributed at irregular intervals along the length of the yarn, and other portions of the multifilament yarn are re-bundled while travelling from the slub-forming device 4 to the take up package 9.

The multifilament yarns usable for the process of the present invention may be selected conventional natural and artificial multifilament yarns. The natural multifilament yarn may be a silk yarn. The artificial multifilament yarn may be a regenerated cellulose multifilament yarn, for example, viscose rayon or cuprammonium rayon yarn, regenerated protein multifilament yarn, semi-synthetic multifilament yarn, for example, cellulose diacetate or cellulose triacetate filament yarn, and synthetic multifilament yarn made of a fiber-forming synthetic polymer, for example, polyester such as polyethylene terephthalate, polybutylene terephthalate, polyoxyethylene benzoate or polyethylene terephthalate-type copolymers containing isophthalic acid, phthalic acid, adipic acid, sebatic acid, diethylene glycol or polyethylene glycol and copolymers of these; polyamide such as nylon 6, nylon 66, nylon 610, nylon 12, polyamide including cyclohexane groups, polyamide including isophthalic acid, phthalic acid or terephthalic acid or these copolymer; polyamidoether; polyolefin such as polyethylene, polypropylene or ethylene-propylene copolymer; and acrylic polymer such as polyacrylonitrile or acrylonitrile copolymer.

It is desirable that the multifilament yarn usable for the present invention be easily opened by the action of the air vortex or turbulent current produced in the slub-forming device. For this purpose firmly twisted multifilament yarns are firmly bonded multifilament yarns with a sizing agent are not suitable because they are difficult to open. However, the firmly twisted and sized multifilament yarns may be used for the process of the present invention if at least one other multifilament yarn which can be easily opened, is used, as a slub-forming yarn, together with them.

Referring to FIG. 1, the feed means 3a and 3b for the multifilament yarn 1 feed the yarn at a constant rate without slippage of the yarn on the feed means. The feed means may be of any type, for example, a pair of nip rollers as shown in FIG. 1, apron rollers or Nelson's rollers.

The winding up means for the slub yarn may be a conventional winder capable of taking up the slub yarn at a desired constant rate. For the process of the present invention, a conventional RT winder having no transverse guide and traveller is preferable rather than a conventional spindle drive winder or QT winder which have the traverse guide and traveller. This is because the slubs formed on the slub yarn of the present invention tend to restrict passage of the yarn through the traverse guide and traveller. This is because the slubs have a larger thickness than that of the original multifilament yarn and, therefore, are frequently caught in the traverse guide and traveller.

The slub-forming device for forming therein the reduced pressure region, will be explained in detail by re-

5  
ferring to FIGS. 2 through 9 of the accompanying drawings.

FIG. 2 shows a longitudinal cross-sectional view of a simple embodiment of the slab-forming device. The slab-forming device 11 has a hollow column 12, a yarn supply end plate 13 and a yarn delivery end plate 15. The yarn supply end plate 13 has a yarn supply hole 14 formed in the center of the plate 13. The yarn delivery end plate 15 has a yarn delivery hole 16 formed in the center of the plate 15. One end of an air suction pipe 17 is connected to a middle portion of the wall of the hollow column 12. The other end of the air suction pipe 17 is connected to a vacuum device (not shown in FIG. 2) such as a vacuum pump.

When the vacuum device is actuated, the pressure of the hollow column 12 is reduced, and air is sucked at a high flow rate from the atmosphere through the yarn supply and delivery holes 14 and 16 into the hollow column 12. The air thus sucked generates under a reduced pressure an air vortex or turbulent current in the hollow column 12.

The multifilament yarn, together with the sucked air, is fed into the hollow column 12 through the yarn supply hole 14 and vigorously agitated by the action of the air current. During the agitating, portions of the multifilament yarn 1 are converted into slubs 7a distributed randomly along the yarn 7.

Sometimes, portions of the yarn 1 are sucked from the hollow column 12 into the air suction pipe 17 and converted into slubs having a relatively long length.

The hollow column 12 may have a circular cross-sectional profile or an irregular cross-sectional profile, for example, square, hexagonal, octagonal and oval cross-sectional profiles.

In FIG. 3, the slab-forming device 21 is similar to the slab-forming device 11 shown in FIG. 2 except that the hollow column 12 is divided into two compartments by an air permeable partition 22. The partition 22 is perforated and has a plurality of small holes 23. The partition 22 is arranged parallel to the yarn travel path from the yarn supply hole 14 to the yarn delivery hole 16, between the yarn travel path and the end of the air suction pipe 17 connected to the wall of the hollow column 12. That is, one of the compartments is connected to the vacuum device (not shown in FIG. 3) through the air suction pipe 17 and the other compartment is connected to the atmosphere through the yarn supply and delivery holes 14 and 16. Only air, and not, the multifilament yarn can pass through the small holes 23 of the partition 22. The perforated partition 22 may be a 20 to 100 mesh net.

When the vacuum device (not shown) is actuated, air is sucked from atmosphere through the yarn supply and delivery holes 14 and 16 into the hollow column 12 at a very high flow rate. A portion of the sucked air collides with the partition 22 and the other portion passes through the small holes 23 of the partition 22. The passing of the sucked air through the small holes 23 of the partition 22 causes suction of the multifilament yarn onto the surface of the partition 22 and the multifilament yarn temporarily stays on the partition surface 22. The collision of a portion of the sucked air with the partition 22 results in very vigorous agitation of the multifilament yarn which has been sucked onto the partition. While in the hollow column 12, the multifilament yarn 1 is prevented by the partition 22 from suction into the air suction pipe 17. This prevention is effective for promoting the formation of relatively uni-

5  
form slubs in length, thickness and distribution. This is because the condition of the multifilament yarn staying in the slab-forming device 21 is relatively uniform throughout the operation time. In the embodiment of the apparatus as shown in FIG. 3, the hollow column preferably has an irregular cross-sectional profile, for example, square, hexagonal and octagonal cross-sectional profiles.

10  
15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415  
8420  
8425  
8430  
8435  
8440  
8445  
8450  
8455  
8460  
8465  
8470  
8475  
8480  
8485  
8490  
8495  
8500  
8505  
8510  
8515  
8520  
8525  
8530  
8535  
8540  
8545  
8550  
8555  
8560  
8565  
8570  
8575  
8580

inside diameter of the yarn storage inner hollow column 42. The yarn travel path passes through the center opening 46 of the air suction member 45. The air suction member 45 is provided with one or more air suction holes 47 through which the center opening 46 is connected to the atmosphere. The air suction hole 47 is formed in such a manner that the longitudinal axis of the air suction hole 47 does not intersect the longitudinal axis of the center opening 46. The air suction holes 47 thus formed are effective for generating a vortex of the sucked air in the slab-forming device 41.

Referring to FIG. 7, the holes 43 are formed through the wall of the yarn storage inner hollow column 42 in such a manner that the longitudinal axes of the holes 43 do not intersect the longitudinal axis of the yarn storage inner hollow column 42. The holes 43 are effective for promoting the formation of vortex of the sucked air in the yarn storage inner hollow column 42. The holes 43 may be formed in such a manner that the longitudinal axes of the holes 43 intersect the longitudinal axis of the yarn storage inner hollow column.

When the vacuum device (not shown in FIG. 5) is actuated, air is sucked from the atmosphere into the slab-forming device 41 through the yarn supply and delivery holes 14 and 16 and the air suction holes 47 of the air suction member 45. The air sucked through the air suction holes 47 and the yarn delivery hole 16 is formed into a vortex in the center opening 46, and further sucked into the air suction pipe 17. The air sucked into the yarn storage inner hollow column 42 through the yarn supply hole 14 is further sucked into the suction pipe 17 through the holes 43 and also the opening 45 and clearance 48. Accordingly, in the yarn delivery end portion of the yarn storage inner hollow column 42, air flows upward from the middle portion thereof and in the yarn supply end portion of the inner hollow column 42, air flows downward from the middle portion. That is, the sucked air in the yarn storage inner hollow column 42 is formed into two currents in opposite directions to each other. Therefore, the middle portion of the yarn storage inner hollow column 42 is reduced into a lower pressure than the other portions. In the middle portion, the turbulent air current is most vigorous. When the multifilament yarn 1 is fed into the yarn storage inner hollow column 42 through the yarn supply hole 14, the yarn 1 is vigorously agitated in the middle portion. While passing through the center opening 46 of the air suction member 45, the agitated yarn 1 is re-bundled by the air vortex.

Referring to FIG. 8, the slab-forming device 51 is provided with an air vortex inner hollow column 52 extending from the air suction member 45 toward the yarn storage inner hollow column 42. The hollow space of the air vortex inner hollow column 52 is connected with the center opening 46 of the air suction member 45. The end of the air vortex inner hollow column 52 facing the open end 44 of the yarn storage inner hollow column 42, is closed with an end member 53 having a funnel-shaped inside surface 54 and a hole 55 through which the yarn travels. Further, the air vortex inner hollow column 52 has a plurality of holes 56 formed in the side walls thereof. Referring to FIG. 9, the holes 56 are formed through the side walls of the air vortex inner hollow column 52 in such a manner that the longitudinal axes of the holes 56 do not intersect the longitudinal axis of the air vortex inner hollow column 52.

The multifilament yarn is vigorously agitated in the middle portion of the yarn storage inner hollow column

42, and travels into the air vortex inner hollow column 52 through the hole 55. The air vortex inner hollow column 52 strengthens the air vortex produced by the air suction member 45. Accordingly, while traveling through the air vortex inner hollow column 52 and the center opening 46 of the air suction member 45, the agitated yarn is re-bundled. That is, the slab-forming device 51 of FIG. 8 is effective for producing a compact slab yarn. The air vortex inner hollow column may be of a circular cross-sectional profile or an irregular cross-sectional profile, for example, square, hexagonal, octagonal and oval cross-sectional profiles.

The hollow column 12 and the yarn storage inner hollow column 42 wherein the slubs are formed, may have an inside wall surface containing sharply edged fine particles. Some of the individual filaments agitated in the slab-forming device come into contact with the abrasive surface containing the sharply edged particles and are broken. The broken filaments form fluffs on the yarn. Therefore, the resultant slab yarn has a spun slab yarn-like appearance but is made of the multifilament yarn.

The abrasive surface carries thereon numerous fine abrasive grains having a high hardness and sharp edges to scratch or break the filaments. The abrasive surface may be an abrasive sheet such as sand paper or sand cloth, on which numerous abrasive grains are fixed with a binder.

The abrasive grains preferably consist of a metallic material such as carbon steel quenched by high frequency induction process, or an inorganic material such as diamond, boron carbide, silicon carbide, crystallized alumina, molten zircon, garnet, jade and rock crystal, silica, molten quartz, orthoclase and apatite, or mixtures of two or more of these materials. The abrasive grains preferably have a size of 16 to 250  $\mu$  and are preferably distributed in a density of 50 grains/cm<sup>2</sup> or more.

The slab-forming devices usable for the present invention are not limited to those as shown in FIGS. 2 through 9. Rather, these FIGS. merely illustrate particular preferred embodiments of the present invention. It will be recognized that variations and modifications of the disclosed apparatus including the rearrangement of parts, lie within the scope of the present invention.

FIGS. 10 and 11 show explanatory views of slab yarns produced by the present invention, respectively. In FIG. 10, the slab is formed from complicitely entangled, intertwined, folded and/or looped individual filaments separated from each other. In FIG. 11, the slab is formed by a portion of the yarn being folded and intertwined with itself.

In the process of the present invention, the pattern of the slab to be produced is in response to condition of the sucked air current under a reduced pressure and the overfeed ratio. The term "overfeed ratio" used here refers to a ratio in percent of the difference between the feed rate and the delivery rate of the multifilament yarn to the delivery rate.

The condition of the sucked air current depends on the type of the slab-forming device, and has an influence upon the configuration and length of the slubs. The overfeed ratio influences the frequency of the slab formation and length of the slab.

In the process of the present invention, the overfeed ratio may be varied within a range of from 5 to 300%. Accordingly, by adjusting the overfeed ratio and selecting the type of the slab-forming device, almost all pat-

terns of slub yarns can be obtained.

Depending upon the overfeed ratio, type of the slub-forming device and degree of vacuum, sometimes, the resultant slub yarn has slubs formed by loosely entangling and intertwining the yarn and/or individual filaments. Such slubs are very bulky. Therefore, in the travelling of the slub yarn, the loosely formed slubs are frequently restricted by the yarn guide in a rewinding, weaving or knitting machine. The interruption results in breakage of the slub yarn. Accordingly, the slub yarn having such loosely formed slubs cannot be used for rewinding, weaving and knitting. In this case, the defect as stated above can be eliminated by the following methods:

1. Firmly re-bundling the slub yarn removed from the slub-forming device by blowing a jet of air onto the slub yarn.

2. Firmly bonding the slub yarn by applying a bonding agent, such as sizing agent and resin.

3. Tightening the slub yarn by passing through a high temperature zone to shrink the looped filaments and loosely entangled yarn and filaments.

Otherwise, in order to produce firmly bundled slub yarn, it is effective to lightly twist the multifilament yarn in a small number of twists before feeding it into the slub-forming device, to lightly interlace the individual filaments by blowing a jet of air onto the yarn before the slub-forming. The twisting and interlacing stated above are effective for controlling the opening of the multifilament yarn.

The multifilament yarn usable for the present invention may be composed of a single multifilament yarn or two or more component multifilament yarns. The component multifilament yarns may be the same as or different from each other. The different component multifilament yarns may be different in type of polymer, denier of the yarn or individual filament, number of individual filaments and type of process applied to the yarn. That is, the multifilament yarn may be a crimped yarn, textured yarn or regular yarn, or a doubled yarn of a crimped or textured yarn and a regular yarn. Also, the multifilament yarn may consist of two or more thermoplastic polymer component yarns different in melting point from each other. The slub yarn produced by the present invention may be further subjected to a crimping or texturing process such as stuffing crimping and false-twisting.

In the case where the slub yarn consists of two or more thermoplastic polymer yarns different in melting point from each other, the slub yarn may be heat treated at a temperature lower than the lighter melting point but not lower than the lower melting point of the yarns. By the heat treatment, the higher melting point yarn is firmly bonded by the melted lower melting point yarn.

As stated hereinbefore, energy efficiency of the process of the present invention is higher than the conventional slub-forming methods wherein a fluid jet is blown onto the yarn, because the slub-forming is effected in a reduced pressure region wherein the yarn and individual filaments can easily move. Further, the apparatus of the present invention involves no twisting means and mechanism for forming slubs at random which are necessary for the conventional slub forming apparatuses. Therefore, the apparatus of the present invention is very simple in structure and of low cost, and can be driven at a very high velocity.

The following examples are presented merely for the purpose of illustrating the present invention.

#### EXAMPLES 1 THROUGH 30

- 5 As shown in Table 1, in Example 1, a polyethylene terephthalate multifilament yarn of 100 denier consisting of 48 filaments (100 d/48 f) was twisted at a twist number of 10 turns per meter (10 T/M). The twisted yarn was processed in the apparatus as shown in FIG. 1 10 having the slub-forming device as shown in FIG. 2 under conditions as shown in Table 1, columns 4, 5, 6 and 7. In Table 1, column 6, the term "overfeed ratio" refers to a ratio in % of the difference between the feed rate and delivery rate of the yarn for the slub-forming device to the delivery rate. The processed yarn had the properties as shown in Table 2. In Table 2, the term "frequency in forming of slub" refers to the number of slubs formed in a 100 m length of the processed yarn. 15 The same procedures as in Example 1 were repeated 20 in Examples 2 through 4, respectively, using the slub-forming device shown in FIGS. 3 through 5, under conditions detailed in Table 1. The properties of the slub-formed yarns in Examples 2 through 4 are shown in Table 2. 25 The same procedures as in Example 1 through 4 were repeated in Examples 5 through 30, under the conditions and using the yarn and the slub-forming device as shown for each example in Table 1. The slub-formed yarns in Examples 5 through 30 had the properties 30 shown in Table 2.

Referring to Tables 1 and 2, the processed yarns in Examples 1, 5, 9, 10, 11, 15, 19 and 23, which had been slub-formed by the slub-forming device of FIG. 2, had slub lengths varying in a wide range.

35 The slub-formed yarns in Examples 2, 6, 12, 16, 20, 24 and 25 using the slub-forming device of FIG. 3 had relatively short and thick slubs. The yarns slub-formed in Examples 3, 7, 13, 17, 21, 26 and 27 using the slub-forming device of FIG. 4 had relatively long and thin 40 slubs. In Examples 4, 8, 14, 18, 22, 28, 29 and 30 using the slub-forming device as shown in FIG. 5, the processed yarns had relatively thin and short slubs which were slightly different, in thickness and appearance, from the non slub-forming portion of the yarn.

45 From Tables 1 and 2, it is clear that the process and apparatus of the present invention are applicable for all types in material of multifilament yarns because neither heat nor chemicals are used for the slub-forming. The patterns of the slubs formed by the process of the present invention vary, in length, thickness and configuration, in response to the type of slub-forming device used. Further, it should be noted that the process of the present invention is applicable to any type in configuration of regular multifilament yarns, textured yarns, composite yarns of regular yarn with textured yarn and composite yarns of two or more same or different types of textured yarns. That is, the patterns of the formed slubs can be varied simply by varying the type of slub-forming device and the slub-forming condition. The 50 slub yarns produced in Examples 1 through 30 were similar in weaving property to the conventional twisted slub yarns, and somewhat poorer than the regular twisted yarns because the slubs sometimes cause breakage of the yarn. The frequency of the yarn breakages depends on the pattern of the slubs. The fabrics produced from the slub yarns of Examples 1 through 30 were all uniform in appearance, having no unevenness in a tortoise-shell pattern or wood grain pattern. These 55 60 65

fabrics each had a very soft feel to the hand because the yarn was not twisted during the slab-forming process. Further, since the regular portions of the slab yarn are somewhat dishevelled in parallel arrangement of the individual filaments by the action of the sucked air current, the fabrics had silk fabric-like luster due to desirable diffused reflection of light at the regular portions of the slab yarns in the fabrics.

Some of the slab yarns in these examples had loops formed by the dishevelled individual filaments in the 10 slubs and the regular portions of the yarns.

Table 2-continued

| Ex. No. | Mean length of slubs (cm) | Largest length of slubs (cm) | Frequency in forming of slubs | Weaving property | Looped filaments on fabric |
|---------|---------------------------|------------------------------|-------------------------------|------------------|----------------------------|
| 10      | 33                        | 82                           | 45                            | normal           | "                          |
| 11      | 25                        | 105                          | 53                            | normal           | "                          |
| 12      | 11                        | 35                           | 85                            | good             | "                          |
| 13      | 23                        | 79                           | 31                            | slightly poor    | negligible                 |
| 14      | 4                         | 16                           | 220                           | good             | slightly noticeable        |

Table 1

| Ex. No. | Starting yarn                                                                     | Slab-forming device | Feed rate (m/min) | Wind up rate (m/min) | Over-feed ratio (%) | Degree of vacuum (mmHg) |
|---------|-----------------------------------------------------------------------------------|---------------------|-------------------|----------------------|---------------------|-------------------------|
| 1       | Polyethylene terephthalate (PET) yarn 100 d/48 f, 10 T/M                          | A                   | 460               | 400                  | 15                  | 45                      |
| 2       | "                                                                                 | B                   | "                 | "                    | "                   | "                       |
| 3       | "                                                                                 | C                   | "                 | "                    | "                   | "                       |
| 4       | "                                                                                 | D                   | "                 | "                    | "                   | "                       |
| 5       | Cellulose diacetate yarn 150 d/30 f, 10 T/M                                       | A                   | 420               | 350                  | 20                  | "                       |
| 6       | "                                                                                 | B                   | "                 | "                    | "                   | "                       |
| 7       | "                                                                                 | C                   | "                 | "                    | "                   | "                       |
| 8       | "                                                                                 | D                   | "                 | "                    | "                   | "                       |
| 9       | Nylon 66 yarn 75 d/36 f 10 T/M                                                    | A                   | 520               | 450                  | 15                  | 50                      |
| 10      | Polyacrylonitrile yarn 150 d/48 f, 15 T/M                                         | A                   | "                 | "                    | "                   | "                       |
| 11      | Cellulose diacetate yarn 150 d/30 f crimped by a gear crimping machine            | A                   | 360               | 300                  | 20                  | 40                      |
| 12      | "                                                                                 | B                   | "                 | "                    | "                   | "                       |
| 13      | "                                                                                 | C                   | "                 | "                    | "                   | "                       |
| 14      | "                                                                                 | D                   | "                 | "                    | "                   | "                       |
| 15      | PET 150 d/30 f false-twisted textured yarn and PET 50 d/24 f, 10 T/M regular yarn | A                   | 455               | 350                  | 30                  | 50                      |
| 16      | "                                                                                 | B                   | "                 | "                    | "                   | "                       |
| 17      | "                                                                                 | C                   | "                 | "                    | "                   | "                       |
| 18      | "                                                                                 | D                   | "                 | "                    | "                   | "                       |
| 19      | PET 50 d/24 f, 10 T/M and cellulose diacetate yarn 100 d/24 f, 60 T/M             | A                   | 495               | 450                  | 10                  | "                       |
| 20      | PET 50 d/24 f, 10 T/M and cellulose diacetate yarn 100 d/24 f, 60 T/M             | B                   | 495               | 450                  | 10                  | 50                      |
| 21      | "                                                                                 | C                   | "                 | "                    | "                   | "                       |
| 22      | "                                                                                 | D                   | "                 | "                    | "                   | "                       |
| 23      | PET 100 d/48 f, 10 T/M regular yarn                                               | A                   | 440               | 400                  | 10                  | 45                      |
| 24      | "                                                                                 | B                   | "                 | "                    | "                   | "                       |
| 25      | "                                                                                 | B                   | 520               | "                    | 30                  | "                       |
| 26      | "                                                                                 | C                   | 440               | "                    | 10                  | "                       |
| 27      | "                                                                                 | C                   | 520               | "                    | 30                  | "                       |
| 28      | "                                                                                 | D                   | 440               | "                    | 10                  | "                       |
| 29      | "                                                                                 | D                   | 520               | "                    | 30                  | "                       |
| 30      | "                                                                                 | D                   | 600               | "                    | 50                  | "                       |

Note: A, B, C and D are slab-forming devices shown in Figs. 2, 3, 4 and 5, respectively.

Table 2

| Ex. No. | Mean length of slubs (cm) | Largest length of slubs (cm) | Frequency in forming of slubs | Weaving property | Looped filaments on fabric | 55 | 15 | 35  | 125 | 63  | slightly poor | "          |
|---------|---------------------------|------------------------------|-------------------------------|------------------|----------------------------|----|----|-----|-----|-----|---------------|------------|
| 1       | 30                        | 108                          | 38                            | normal           | slightly noticeable        | 60 | 16 | 10  | 30  | 135 | normal        | "          |
| 2       | 15                        | 25                           | 70                            | good             | noticeable                 | 17 | 28 | 103 |     | 39  | slightly poor | negligible |
| 3       | 31                        | 125                          | 20                            | slightly poor    | negligible                 | 21 | 17 | 120 |     | 57  | normal        | negligible |
| 4       | 5                         | 10                           | 180                           | good             | very noticeable            | 22 | 4  | 13  | 65  | 28  | good          | negligible |
| 5       | 35                        | 100                          | 51                            | normal           | slightly noticeable        | 23 | 13 | 65  | 25  | 30  | normal        | negligible |
| 6       | 21                        | 40                           | 98                            | normal           | noticeable                 | 24 | 7  | 26  | 128 | 152 | good          | negligible |
| 7       | 63                        | 150                          | 39                            | normal           | noticeable                 | 25 | 10 | 30  | 135 | 32  | normal        | negligible |
| 8       | 5.8                       | 15                           | 250                           | good             | noticeable                 | 26 | 15 | 128 |     | 92  | slightly poor | negligible |
| 9       | 28                        | 76                           | 52                            | normal           | slightly                   | 27 | 20 | 135 |     | 28  | good          | negligible |
|         |                           |                              |                               |                  |                            | 28 | 5  | 8   | 150 | 150 | slightly      | negligible |

Table 2-continued

| Ex.<br>No. | Mean<br>length<br>of slubs<br>(cm) | Largest<br>length<br>of slubs<br>(cm) | Frequency<br>in forming<br>of slubs | Weaving<br>property | Looped<br>filaments on<br>fabric     |
|------------|------------------------------------|---------------------------------------|-------------------------------------|---------------------|--------------------------------------|
| 29         | 6                                  | 13                                    | 293                                 | good                | noticeable                           |
| 30         | 6                                  | 65                                    | 100                                 | normal              | noticeable<br>slightly<br>noticeable |

## EXAMPLES 31 THROUGH 33

In Example 31, the same procedures as in Example 1 were repeated using the same apparatus as shown in FIGS. 1 and 2 except that an interlace nozzle was arranged between the slab-forming device and the delivery roller 8 and compressed air of a 3 kg/cm<sup>2</sup> pressure was ejected onto the slab-formed yarn through the interlace nozzle.

In Example 32, the same procedures as in Example 31 were repeated using, instead of the interlace nozzle, a rotatable sizing roller located between slab-forming device and the delivery roller 8. A lower portion of the sizing roller was immersed in a bath containing an aqueous solution of 3% by weight of polyvinyl alcohol. The slab-formed yarn delivered from the slab-forming device was brought into contact with an upper portion of the sizing roller, carrying on its periphery surface a polyvinyl alcohol solution, and sized.

In Example 33, the same procedures as in Example 31 were repeated using, instead of the interlace nozzle, a hot plate of a 1 m length placed between the slab-forming device and the delivery roller. The hot plate was heated at a temperature of 230°C, and the slab-formed yarn delivered from the slab-forming device came into contact with the heating surface of the hot plate. The resultant slab yarns in Examples 31 through 33 were remarkably improved in the bundling of the individual filaments in the slab portions and the regular portions of the slab yarns. That is, in these slab yarns disheveling of the individual filaments was prevented. This is similar to the conventional twisted slab yarns.

The slab yarn of Example 31 had small loops of the filaments. However, the processability in weaving and knitting of the slab yarn was similar to that of the regular multifilament yarns. The slab yarns of Examples 32 and 33 had much less filament loops and were similar in processability to the regular yarns.

Further, it should be noted that even in the cases where the interlace nozzle, sizing roller or hot plate was located between the slab-forming device was the delivery roller to bundle the individual filaments in the slab 5 yarn, the resultant slab yarn had no change in slab pattern, that is, frequency in slab forming and length and thickness of the slubs.

Additionally, the same procedures as in Examples 31 through 33 were repeated using the same starting yarn 10 under the same process conditions as those in Examples 2, 3, 4, 19, 20, 21 or 22. All of the procedures were carried out without difficulty, and the resultant slab 15 yarns were improved in bundling of the individual filaments.

## EXAMPLES 34 THROUGH 41

The same slab yarns as produced in Examples 1 through 4 and 19 through 22 were crimped using a gear crimping machine having a heater device located up-

20 stream of the crimping gear. The crimped slab yarns were used to produce fabrics. The resultant fabrics had a high bulkiness and very soft feel to the hand. The heater device located upstream of the crimping gear was effective for improving the bundling of the individual filaments in the slab yarns. Therefore, the crimped 25 slab yarns were woven into uniform fabrics without difficulty.

The same procedures as in Examples 34 through 41 were repeated using, instead of the gear crimping machine, a frictional false-twisting device. The resultant 30 fabrics were highly bulky and very soft. The false-twisting device was provided with a heater located upstream from a friction drive means. The heater was effective for bundling the individual filaments in the slab yarns.

## EXAMPLES 42 THROUGH 49

An interlace nozzle was located upstream of the feed roller in the apparatus shown in FIG. 1. In Example 42, the same procedures as in Example 1 were repeated

40 using the above-mentioned apparatus. Before the slab-forming step, the starting yarn was lightly bundled by the action of a compressed air current spouted through the interlace nozzle under a pressure of 0.5 kg/cm<sup>2</sup>. The processed yarn had the properties as shown in 45 Table 3.

In Examples 43 through 49, the same procedures as in Examples 2 through 4 and 19 through 22, respectively, were repeated using the above-mentioned apparatus. The properties of the resultant slab yarns are 50 shown in Table 3.

Table 3

| Ex.<br>No. | Starting yarn<br>and process<br>conditions | Slub-yarn                             |                                       |                                  |                     |                 |
|------------|--------------------------------------------|---------------------------------------|---------------------------------------|----------------------------------|---------------------|-----------------|
|            |                                            | Mean<br>length<br>of<br>slubs<br>(cm) | Largest<br>length<br>of slubs<br>(cm) | Frequency<br>in slab-<br>forming | Weaving<br>property | Loop<br>forming |
| 42         | as Example 1                               | 41                                    | 115                                   | 26                               | slightly<br>poor    | ordinal         |
| 43         | as Example 2                               | 26                                    | 41                                    | 53                               | normal              | ordinal         |
| 44         | as Example 3                               | 40                                    | 153                                   | 14                               | slightly<br>poor    | less<br>ordinal |
| 45         | as Example 4                               | 6                                     | 19                                    | 113                              | normal              | less            |
| 46         | as Example 19                              | 15                                    | 38                                    | 19                               | slightly<br>poor    | ordinal         |
| 47         | as Example 20                              | 10                                    | 37                                    | 24                               | normal              | less            |
| 48         | as Example 21                              | 20                                    | 135                                   | 13                               | slightly<br>poor    | ordinal         |
| 49         | as Example 22                              | 5                                     | 15                                    | 125                              | good                | less<br>ordinal |

## 15

The spouting of the compressed air resulted in slightly bundling the individual filaments in the starting yarn. The bundling caused difficulty in the opening of the individual filaments in the slab-forming step. Less opening of the individual filaments resulted in less entanglements, interwindings and loopings of the individual filaments. Accordingly, Table 3 shows that the resultant slab yarns had less frequency of slab-forming and larger slab length than those in Examples 1 through 4 and 19 through 22. Further, the loopformation in Examples 42 through 49 was less than in the corresponding foregoing examples. Therefore, the slab yarns obtained in the present examples had regular (non slab-formed) portions similar in appearance to the starting yarn.

## EXAMPLE 50

A hot plate of a 1 m length was inserted between the slab-forming device and the delivery roller in apparatus shown in FIG. 1. The hot plate was maintained at a temperature of 170°C to heat the slab yarn delivered from the slab-forming device.

A polyethylene terephthalate multifilaments yarn of a 300 denier consisting of 36 filaments and having a twist number of 10 T/M was doubled with a polypropylene yarn of 30 denier consisting of 7 filaments and having a twist number of 10 T/M and the doubled yarn was fed into the above-stated apparatus having slab-forming device as shown in FIG. 5 to convert it into a slab yarn. The fed doubled yarn was processed under the following conditions.

|                         |           |
|-------------------------|-----------|
| Feed rate               | 345 m/min |
| Wind-up (delivery) rate | 300 m/min |
| Degree of vacuum        | 50 mmHg   |
| Heater temperature      | 170°C     |

When the doubled yarn came into contact with the heater plate, the polypropylene yarn was melted in parts and bonded the individual polyethylene terephthalate filaments and the remaining polypropylene filaments in the slab yarn. The loops formed on the slab yarn were shrunk by the contact with the heater plate. Accordingly, the resultant slab yarn has a high processability in winding, weaving and knitting.

The same procedures as in the present example were repeated using, instead of the slab-forming device of FIG. 5, the slab-forming device of FIGS. 2, 3 and 4. The resultant slab yarns were similar in processability to the yarn in the present example.

What we claim is:

1. A process for continuously producing slab yarns comprising the steps of:

providing a reduced pressure region in a closed hollow column and connected to the atmosphere through a yarn supply hole at an end of said column and a yarn delivery hole located at an opposite end of said column, by sucking air from the atmosphere through said region;

feeding a multifilament yarn into said reduced pressure region through said yarn supply hole at predetermined feed rate while sucking air through said region;

agitating said fed multifilament yarn in said reduced pressure region by action of the sucked air current in order to convert portions of said multifilament yarn into slubs; and

## 16

delivering said resultant slab yarn from said reduced pressure region through said yarn delivery hole at a delivery rate lower than said feed rate.

2. A process as claimed in claim 1, wherein said fed multifilament yarn is sucked onto an air-permeable surface provided within said reduced pressure region.

3. A process as claimed in claim 2, wherein said fed multifilament yarn temporarily stays on said air-permeable surface.

4. A process as claimed in claim 1, wherein said sucked air is formed into two currents in opposite directions to each other within said reduced pressure region.

5. A process as claimed in claim 1, wherein said slab yarn delivered from said reduced pressure region is rebundled by the action of an air jet blown onto the slab yarn.

6. A process as claimed in claim 1, wherein said slab yarn delivered from said reduced pressure region is bonded by applying a bonding agent to the slab yarn.

7. A process as claimed in claim 1, wherein said slab yarn delivered from said reduced pressure region is tightened by heating it at a temperature at which the looped or loosely entangled individual filaments shrink.

8. A process as claimed in claim 1, wherein said multifilament yarn is lightly bundled before feeding it into said reduced pressure region.

9. A process as claimed in claim 1, wherein said multifilament yarn is a crimped or textured yarn.

10. A process as claimed in claim 1, wherein said multifilament yarn consists of two or more component multifilament yarns.

11. A process as claimed in claim 10, wherein said component yarns are the same.

12. A process as claimed in claim 10, wherein said component yarns are different from each other.

13. A process as claimed in claim 12, wherein said component yarns are one or more crimped multifilament yarns and one or more regular multifilament yarns.

14. A process as claimed in claim 12, wherein said component yarns are thermoplastic polymer multifilament yarns different in melting point from each other.

15. A process as claimed in claim 14, wherein said slab yarn consisting of said thermoplastic polymer multifilament yarns different in melting point from each other, is heat treated at a temperature lower than the higher melting point but not lower than the lower melting point of said thermoplastic polymer multifilament yarns.

16. A process as claimed in claim 1, wherein a ratio of difference between said feed rate and said delivery rate to said delivery rate is in a range from 5 to 300%.

17. A process as claimed in claim 1, wherein said yarn is, after slab-forming, further re-bundled within said reduced pressure region by action of a vortex of the sucked air.

18. A process as claimed in claim 1, wherein said yarn travels upward.

19. An apparatus for continuously producing a slab yarn from a multifilament yarn, comprising:

a slab-forming device comprising a closed hollow column having a yarn supply plate located at an end of said column and having a yarn supply hole formed thereon and a yarn delivery plate located at an opposite end of said column and having a yarn delivery hole formed thereon;

feed means for feeding a multifilament yarn at a predetermined feed rate into said slab-forming device through said yarn supply hole; delivery means for delivering a slab-yarn at a predetermined delivery rate lower than said feed rate from said slab-forming device through said yarn delivery hole, and;

means for sucking air from the atmosphere through said slab-forming device, said means being connected to the periphery of said hollow column.

20. The apparatus of claim 19 wherein said means for sucking air is connected to the periphery of said hollow column by a pipe.

21. An apparatus as claimed in claim 20, wherein said pipe is provided with an air permeable partition located therein.

22. An apparatus as claimed in claim 19, wherein said hollow column has a circular cross-sectional profile.

23. An apparatus as claimed in claim 19, wherein said hollow column has an irregular cross-sectional profile.

24. An apparatus as claimed in claim 19, wherein said hollow column of said slab-forming device is divided into two compartments with an air permeable partition disposed in parallel to the yarn travel path from the yarn supply hole to the yarn delivery hole, between the yarn travel path and the entrance of said air suction means.

25. An apparatus as claimed in claim 24, wherein said hollow column has a square cross-sectional profile.

26. An apparatus as claimed in claim 19, wherein said hollow column of said slab-forming device has a yarn storage inner hollow column located therein and surrounding the yarn travel path between said yarn supply hole and the yarn delivery hole, said yarn storage inner hollow column having a yarn supply end connected to the yarn supply end plate of said hollow column, the other end opening in said hollow column and

a plurality of small holes formed on the yarn supply end portion thereof.

27. An apparatus as claimed in claim 26, wherein said small holes on said inner hollow column are formed in such a manner that the longitudinal axes of said holes do not intersect the longitudinal axis of said yarn storage inner hollow column.

28. An apparatus as claimed in claim 26, wherein said small holes on said inner hollow column are formed in such a manner that the longitudinal axes of said holes intersect the longitudinal axis of said yarn storage inner hollow column.

29. An apparatus as claimed in claim 26, wherein said hollow column further comprises an air suction member located between said yarn delivery end plate and said yarn storage inner hollow column and having a center opening and one or more air suction holes through which said center opening is connected to atmosphere, said air suction holes being formed in such a manner that the longitudinal axes of said air suction holes do not intersect with the longitudinal axis of said center opening.

30. An apparatus as claimed in claim 29, wherein said hollow column of said slab-forming device is further provided with an air vortex inner hollow column extending from said air suction member toward said yarn storage inner hollow column and surrounding said yarn travel path, said air vortex inner hollow column having a plurality of small holes formed on its periphery in such a manner that the longitudinal axes of the holes do not intersect with the longitudinal axis of the air vortex inner hollow column, and a hole formed on its one end facing said yarn storage inner hollow column.

31. An apparatus as claimed in claim 26, wherein said yarn storage inner hollow column has an inside wall surface containing sharply edged fine particles.

32. An apparatus as claimed in claim 19, wherein said hollow column has an inside wall surface made of sharply edged fine particles.

\* \* \* \* \*